

# UNITED STATES PATENT OFFICE.

BRUCE P. JOHNSON, OF MIDVALE, UTAH, ASSIGNOR TO HIMSELF, CLARENCE E. MATTHEWS, AND WILLIAM WATERS, ALL OF MIDVALE, UTAH.

## SHOE-DRESSING.

1,370,819.

Specification of Letters Patent.

Patented Mar. 8, 1921.

No Drawing.

Application filed April 19, 1920. Serial No. 375,080.

To all whom it may concern:

Be it known that I, BRUCE P. JOHNSON, a citizen of the United States, residing at Midvale, in the county of Salt Lake and 5 State of Utah, have invented certain new and useful Improvements in Shoe-Dressings, of which the following is a specification.

This invention relates to certain improvements in shoe dressings and has relation 10 more particularly to a dressing especially adapted for use in connection with white shoes, and it is an object of the invention to provide a novel and improved dressing of 15 this general character which, when applied to the shoe, causes a smooth hard finish which will not rub off.

My improved dressing, as herein embodied, comprises the following admixture:

|    |                     |             |
|----|---------------------|-------------|
| 20 | Zinc oxid C. P.     | 16 oz.      |
|    | Gypsum (powdered)   | 6 oz.       |
|    | Best furniture glue | 3 oz.       |
|    | Ammonia             | 1 fluid oz. |
| 25 | Water               | 1 gal.      |
|    | Blue                | A trace.    |

The zinc oxid serves as a base for the dressing and the combination of the zinc oxid with the gypsum causes a smooth hard

finish, when the dressing is applied to the 30 shoe, which will not rub off. This combination also results in a clear white effect.

The ammonia is added to the mixture for cleaning and bleaching is effected by the slight trace of blue comprised in the mixture. The glue serves as a binder and operates to prevent the dressing, when applied, from rubbing off. By the use of water, the dressing is substantially liquid.

I claim:—

1. A shoe dressing comprising a mixture in water of zinc oxid, gypsum, glue and ammonia, the zinc oxid constituting the major portion of the ingredients other than the water.

2. A shoe dressing comprising a mixture in water of zinc oxid, gypsum, glue and ammonia, the zinc oxid constituting the major portion of the ingredients other than the water, and a trace of blue.

3. A shoe dressing comprising zinc oxid 16 oz., gypsum (powdered) 6 oz., best furniture glue 3 oz., ammonia 1 fluid oz., water 1 gal., blue, a trace.

In testimony whereof I hereunto affix my 55 signature.

BRUCE P. JOHNSON.